

Patented Oct. 9, 1923.

1,470,225

## UNITED STATES PATENT OFFICE.

*Aldehyde*  
*Corrosion*  
*Inhibitors*

HARRY N. HOLMES, OF OBERLIN, OHIO.

## REMOVAL OF SCALE AND RUST FROM IRON AND STEEL.

No Drawing.

Application filed January 17, 1921. Serial No. 437,995.

To all whom it may concern:

Be it known that I, HARRY N. HOLMES, a citizen of the United States, residing at Oberlin, in the county of Lorain and State 5 of Ohio, have invented certain new and useful Improvements in Removal of Scale and Rust from Iron and Steel, of which the following is a specification.

This invention relates to the removal of 10 scale and rust from iron or steel. The invention is particularly applicable for the pickling of iron or steel wire or sheets in mill practice, but is also useful in many other ways, such as for cleaning or freeing 15 iron or steel in any form from rust or oxides, or for removing scale such as boiler scale or the like from sheets or tubes.

One important feature of the invention is the provision of a pickling bath of proper 20 composition and strength and its use under such conditions as will very materially inhibit if not wholly prevent any attack of the iron or steel base by the pickling bath, but without material inhibition of the attack of 25 the bath on rust, or oxides or scale to be removed.

According to my invention the metal is pickled in a bath of suitable acid containing 30 a proper quantity of the inhibiting agent, which may be one of the aldehydes. The presence of a relatively small quantity of an aldehyde in an acid solution is found to inhibit greatly or prevent any attack of the acid upon the base metal but not to prevent 35 or inhibit its attack upon oxides, carbonates, or like materials, such as rust or scale. If the acid solution is sufficiently strong the inhibiting agent, such as an aldehyde, is effective at temperatures above normal or at 40 atmospheric, such as temperatures up to 50° C. or even 80° C., so that according to common mill practice the bath may be used at temperatures above normal with a very material increase above normal in the rate of 45 rust or scale removal, whereas if the acid is weak the inhibiting agent appears to lose its effectiveness above normal temperatures. Consequently relatively strong acid solutions are preferable, although no additional expense in the acid is entailed because the acid attacks the rust or scale and is ineffective 50 upon the base metal.

The acid may be of any of the ordinary acids commonly used for pickling purposes 55 but also is naturally an acid which does not

re-act with the aldehyde. For this reason nitric or other so-called oxidizing acids are not suitable for use, as they probably attack the aldehyde and so oxidize it as to minimize or destroy its inhibiting effect. Examples of 60 suitable acids are sulphuric, hydrochloric, phosphoric, and even acetic or some of the similar weaker or organic acids, although these weaker acids would probably not be sufficiently effective for commercial mill 65 practice.

The acid used can be of any suitable strength with due regard to the facts above noted, to-wit, the loss of effectiveness of the inhibiting agent at higher temperatures 70 when the acid is relatively weak. In practice I have produced useful effects with sulphuric acid solutions made up in the proportions of eleven parts of water to one part of commercial concentrated sulphuric acid 75 by volume. With such solutions containing the inhibiting agent hereafter referred to there is no appreciable effect of the acid upon the base metal. While the oxide or scale is attacked and removed the rate of 80 attack is probably too slow for ordinary mill practice and at higher temperatures, say above 40° or 50° C. the inhibiting effect decreases so as to be practically nil. For 85 these reasons I prefer to use an acid of approximately the strength of one part of acid to five of water by volume. With this solution the inhibiting effect is not only pronounced when the solution is cold or at normal temperatures, but is also so pronounced 90 as to be of practically full value at the temperatures used in mill practice, say 80° C. Hydrochloric acid solutions can be used in various strengths, for example, one volume of commercial concentrated acid to one 95 volume of water, the inhibiting effect being maintained at the higher temperature noted.

The inhibiting agent may be any of the aldehydes but of course is chosen with regard to the cost of material. Good effects 100 have been noted with formaldehyde (the so-called 40% "formalin" solution) benzaldehyde, furfural and acetaldehyde. Acetaldehyde being very volatile would probably be used as the solid, aldehyde ammonia. 105 Other aldehydes are also probably useful. Referring particularly to formaldehyde I find that this material is effective in a pickling bath in relatively small quantities. For example, in a sulphuric acid bath of the dilu- 110

tion of five parts of water to one of commercial concentrated acid by volume the "formalin" solution above referred to may be added in the proportion of as low as one-fifth of one per cent by volume. Larger amounts than this may be employed if desired, but without appearing to materially affect or improve the inhibiting effects, so that additional material is to some extent 10 wasted.

My improved pickling bath enables a base of iron or steel in the form of wire, sheets or the like to be readily and quickly freed of rust, oxide, scale or carbonates by a treatment that can be carried on with as great 15 rapidity as the process, as now in use, but without danger of material attack upon the material. The invention therefore involves a material saving not only in the bath but 20 also in the base metal.

What I claim is:

1. The method of removing rust or scale from iron or steel, consisting in pickling the

same in an acid bath containing at least one-fifth of 1% by volume of an aldehyde to 25 inhibit the attack of the acid upon the base metal.

2. The method of removing rust or scale from iron or steel, consisting in pickling the same in an acid bath containing at least one-fifth of 1% by volume of formaldehyde to 30 inhibit the attack of the acid upon the base metal.

3. The method of removing rust or scale from iron or steel consisting in pickling the same in a bath of sulphuric acid containing at least one-fifth of 1% by volume of an 35 aldehyde.

4. The method of removing rust or scale from iron or steel consisting in pickling the same in a bath of sulphuric acid containing at least one-fifth of 1% by volume of formaldehyde. 40

In testimony whereof I hereby affix my signature.

HARRY N. HOLMES.